

[54] NOVEL EFFECT YARNS AND PROCESS  
FOR PRODUCING THE SAME[75] Inventors: Alexandre Boutonnet, Dommartin;  
Georges Clavelet; Gilbert Morieras,  
both of Lyon, all of France

[73] Assignee: Societe Rhodiacetate, Paris, France

[22] Filed: Nov. 18, 1971

[21] Appl. No.: 200,104

## [30] Foreign Application Priority Data

Nov. 18, 1970 France ..... 70.41663

[52] U.S. Cl. 57/140 BY, 57/157 TS, 161/175

[51] Int. Cl. D02g 3/04, D02g 1/02

[58] Field of Search 57/157 MS, 140 BY, 157 TS,  
57/140 R, 157 R; 161/175

## [56] References Cited

## UNITED STATES PATENTS

3,001,358 9/1961 Mayner ..... 57/140 R  
3,058,291 10/1962 Heberlein et al. ..... 57/140 R

|           |         |                         |             |
|-----------|---------|-------------------------|-------------|
| 3,061,998 | 11/1962 | Bloch .....             | 57/140 BY   |
| 3,251,181 | 5/1966  | Breen et al.....        | 57/140 R    |
| 3,472,017 | 10/1969 | Nakayama et al.....     | 57/140 BY   |
| 3,498,043 | 3/1970  | Moffett, Jr. et al..... | 57/140 R    |
| 3,553,953 | 1/1971  | Ponson.....             | 57/140 R    |
| 3,616,167 | 10/1971 | Gosden.....             | 57/140 BY X |

## FOREIGN PATENTS OR APPLICATIONS

1,045,990 10/1966 Great Britain ..... 57/157 R

Primary Examiner—John W. Huckert

Assistant Examiner—Charles Gorenstein

Attorney, Agent, or Firm—Sherman and Shalloway

## [57] ABSTRACT

Effect yarns having an irregular and twisted surface formed from at least two components having different physical properties, at least one of which is a thermoplastic material which are intermittently bonded to form the effect. These effect yarns are produced by heating the yarns to soften at least one component and twisting and untwisting the softened yarns.

13 Claims, 15 Drawing Figures



Fig. 1.Fig. 2.Fig. 3.

PATENTED AUG 13 1974

3,828,542

SHEET 2 OF 3

Fig. 4.



Fig. 5.



Fig. 6.



Fig. 7.



Fig. 8.



Fig. 9.



Fig. 10.



PATENTED AUG 13 1974

3,828,542

SHEET 3 OF 3

Fig. 11.



Fig. 12.



Fig. 13.



Fig. 14.



Fig. 15.



## NOVEL EFFECT YARNS AND PROCESS FOR PRODUCING THE SAME

The present invention relates to an effect yarn and a process for producing such a yarn.

There are a number of prior art processes for obtaining yarns having a high twist by winding, using a single or double twist spindle. However, throwing is a slow process and the production speeds are lowered if a higher twist is the desired. It has also been proposed to manufacture false twist yarns having high elasticity at greater speeds. However, in these processes yarns having high bulk and/or high elasticity are obtained.

The cohesion of the filaments which comprise a yarn can be increased by various processes, especially by mechanical or pneumatic means. However, these processes generally produce yarns having insufficient compactness for certain applications.

Furthermore, yarns having a high residual twist have been obtained by various processes such as twist accumulation, twist packing and pneumatic false twisting. Here again it is difficult to obtain really compact yarns having the appearance of a monofilament.

The process of the present invention provides a multi-filament yarn with an irregular surface and having a twisted appearance. The multi-filament yarn has at least two filaments, each filament has at least two constituents with different softening temperatures and/or degradation temperature, at least one component being thermoplastic, so that at least some of the filaments are bonded to one another at least at some points along the length of the yarn, in order to provide the surface of the yarn with helical portions of random length, direction and pitch.

The process of the present invention generally comprises feeding a multi-component yarn through a heating zone and then passing the heated yarn through a false twister to twist and untwist the yarn.

It is therefore a primary object of the present invention to provide a process for producing fancy effect yarns.

It is a further object of the present invention to provide a fancy effect multi-filament yarn which is compact and appears to be monofilament yarn.

It is a still further object of the present invention to provide compact multi-filament yarns having an uneven surface and a twisted appearance.

It is a still further object of the present invention to provide a multi-filament yarn wherein the yarn comprises filaments having different thermal and degradation characteristics.

It is a still further object of the present invention to provide a multi-filament yarn wherein the filaments are intermittently bonded to each other.

It is a still further object of the present invention to provide a process for producing multi-filament effect yarns by heating the multi-filaments and subsequently twisting and untwisting the yarns.

Still further objects and advantages of the effect yarns and process for producing the same of the present invention will become more apparent from the following more detailed description thereof.

The multi-filament effect yarns of the present invention comprise at least two filaments having components with differing physical properties, these filaments being intermittently bonded to each other and presenting the

helical appearance of random length, direction and pitch.

The present invention also provides a process for obtaining an effect yarn comprising heating a multi-filament yarn, each filament having at least two components of different softening temperatures and/or degradation temperatures, at least one of said components being thermoplastic to a setting temperature at least equal to the softening temperature of the constituent having the lowest softening temperature, twisting the heated yarn and untwisting the twisted yarn.

The multi-filament yarn of the present invention may be a yarn formed of filaments having different properties, which filaments may or may not be thermoplastic polymers or a yarn formed of at least two identical filaments, each filament having at least two components, arranged coaxially or non-coaxially, such as in a side-by-side relation, sheath-core, etc. when sheath-core filaments are used, the softening temperature of the sheath must be less than the core.

Furthermore, this yarn can contain filaments which possess different physical characteristics or properties, for example elongation, tensile strength or shrinkage, which gives the yarn an additional fancy effect, such as improved bulk. The yarn can consist of continuous filaments or discontinuous filaments such as spun fibres, rovings or ribbons.

Generally, at least a part of at least some of the filaments are welded to one another within a given section of yarn. According to a particular embodiment of the invention, at least a certain number of strands are welded together only at certain points spaced along the length of the yarn and define intermittent free portions which produce an effect. These free portions can be broken by passing the yarns over an abrasive surface, blade, grinding surface, etc., and thus form a yarn having a "spun yarn" appearance.

The novel yarns and process for producing the same will be more readily understood with reference to the following illustrative drawings, in which:

FIG. 1 is a diagrammatic view of a device for the manufacture of a yarn according to the invention, wherein the false-twisting treatment is carried out continuously.

FIG. 2 is a further embodiment of a device for carrying out the process according to the invention with a second heat treatment, after the false-twisting treatment which is carried out continuously.

FIG. 3 diagrammatically represents a device for carrying out the process wherein the false-twisting treatment is carried out discontinuously.

FIGS. 4 to 15 represent yarns obtained in accordance with the examples of carrying out the process according to the invention.

As shown in FIG. 1, a yarn 1 is drawn from a cop 2 and successively passes over a hook 3, a direction-changing guide 4, a tension pulley 5 and a first feed device 6. The yarn then passes through a heating element 7 and then through a false-twist spindle 8, over a second feed device 9 and over a guide 10 before being wound up on a bobbin 11 by a conventional winding system.

The arrangement shown in FIG. 2 is similar to that in FIG. 1, except that the yarn passes downstream of the false-twist spindle 8, through a second heating element 12 before being wound up.

According to FIG. 3, the yarn 13 drawn from a bobbin 14 which freely rotates is given a certain twist, and then passes over a balloon guide 15 and then over a heating plate 16. The yarn is thereafter wound up on a bobbin 18 while being guided by a guide 17 by a conventional reciprocating winding system. Subsequently, the yarn may be untwisted by a similar unwinding step or other conventional twisting process.

The setting temperatures of heating elements 7 and 12 generally can vary from 150° to 300°C and preferably is regulated at a temperature at most equal to a temperature which does not significantly affect the textile characteristics of the constituent having the highest softening temperature.

Although the process may be conducted continuously or discontinuously, preferably, the twisting-setting-untwisting operation should be carried out continuously as shown in FIGS. 1 and 2.

It is possible to obtain a yarn according to the process of the present invention which possesses certain specific effects or characteristics such as flexibility, elasticity, appearance and handle, by varying the composition of the yarn and the treatment conditions. Thus, the heat treatment is generally applied to the yarn continuously, for example, by passing the yarn over a heating plate or through an oven. However, where it is desired to achieve a special effect, a localized heat treatment at various points can be achieved by means of a device for intermittent contact with a heating element.

It is also possible to vary the characteristics of the yarn, for example, the handle, by subjecting it continuously to a more or less rapid cooling between the heat treatment and the twisting-untwisting device. Advantageously, a second heat treatment can be carried out downstream of the twisting-setting-untwisting operation as shown in FIG. 2 so as to increase the fancy effect of the yarn, especially to improve its bulk.

Furthermore, the yarn according to the invention can be subjected to any other customary treatment for the purpose of modifying its characteristics for special applications. Thus, this yarn can be subjected to a treatment which allows the free portions, which appear according to a special form of the invention, to be broken, for example, by sanding, abrasion and the like.

The process according to the invention produces yarns at an advantageous industrial cost, these yarns being perfectly suitable for various applications such as woven fabrics, voile and the like.

Filaments suitable for use in forming the effect yarns of the present invention include thermoplastic fibers such as those produced from polyamides, such as polyhexamethylene adipamide, poly( $\epsilon$ -caprolactam), polyhexamethylene sebacamide, poly (9-aminononanoic acid), poly(11-aminoundecanoic acid), poly lauric lactam, copolymers of any of the above polyamides, polyesters such as those produced by condensing a glycol such as, ethylene, propylene, diethylene, dipropylene or butylene glycol with an acid or anhydride such as adipic acid, azelaic acid, terephthalic acid or phthalic anhydride, e.g., polyethylene terephthalic, polyolefins such as polyethylene, propylene, etc., vinyl polymers such as polyvinyl chloride, polyvinylidene chloride, polyvinyl alcohol, polyacrylonitrile, etc.

The process and product of the present invention will now be illustrated by means of the following specific examples which are for illustration only and not to be taken as limiting the scope of the present invention. In

the following examples, all parts and percentages are by weight and all temperatures are in degrees centigrade.

#### EXAMPLE 1

A coaxial bi-component yarn of 190 dtex/32 filaments is treated in accordance with the process shown diagrammatically in FIG. 1. Each filament comprises in the weight ratio of 80/20:

- 10 i. a copolyamide containing 60 percent of polyhexamethylene adipamide and 40 percent of poly( $\epsilon$ -caprolactam) having a melting point of 180°C, forming the sheath of the yarn; and
- 15 ii. polyhexamethylene adipamide having a relative viscosity of 36 and melting point of about 260°C, forming the core of the yarn.

The yarn passes through an oven heated to 235°C at a speed of 27 m/minute and then into a conventional mechanical false-twist spindle rotating at 50,000 revolutions per minute; the yarn then has a theoretical twist of about 1,800 turns/meter.

The yarn is wound at a speed substantially the same as the speed of travel of the yarn through the oven.

The yarn thus obtained has the appearance of a single filament yarn, the filaments being tightly stuck to each other, its appearance being illustrated in FIG. 4.

#### EXAMPLE 2

A bi-component yarn identical to that of Example 1 is treated in accordance with the same process under the following working conditions:

|    |                                  |                           |
|----|----------------------------------|---------------------------|
| 35 | Oven temperature                 | 220°C                     |
|    | Speed of travel through the oven | 28 m/minute               |
|    | Speed of rotation of the spindle | 28,000 revolutions/minute |
|    | Theoretical twist of the yarn    | 1,000 turns/meter         |

FIG. 5 illustrates the yarn obtained, which is less compact than Example 1 since it is of lower twist, but the filaments in it are again stuck to one another.

#### EXAMPLE 3

The same yarn as in Example 1 is subjected to the same process, under conditions identical to those of Example 2, but inserting a controlled cooling treatment of the yarn on a brass block between the oven and the spindle.

A slight detachment of the free portions is thus obtained, as is illustrated in FIG. 6.

#### EXAMPLE 4

The same yarn as in Example 1 is subjected to the following working conditions:

|    |                                  |                           |
|----|----------------------------------|---------------------------|
| 55 | Oven temperature                 | 240°C.                    |
|    | Speed of travel through the oven | 41 m/minute               |
|    | Speed of rotation of the spindle | 74,000 revolutions/minute |
|    | Theoretical twist of the yarn    | 1,800 turns/meter         |

The yarn obtained according to this example has a more irregular surface than that obtained in Example 1 and its appearance is illustrated in FIG. 7.

#### EXAMPLE 5

The same yarn as in Example 1 is treated, but in ac-

cordance with the process shown diagrammatically in FIG. 2, and under the following conditions:

|                                              |                           |
|----------------------------------------------|---------------------------|
| Oven temperature                             | 240°C.                    |
| Speed of travel of the yarn through the oven | 59 m/minute               |
| Speed of rotation of the spindle             | 74,000 revolutions/minute |
| Theoretical twist of the yarn                | 1,250 turns/meter         |

Thereafter the yarn is subjected to a second heat treatment by passing it through a second oven heater to 240°C.

A yarn with very long free portions, having the appearance shown in FIG. 8, is thus obtained.

#### EXAMPLE 6

The same yarn as in Example 1 is used and is treated in accordance with the process shown diagrammatically in FIG. 2, under the following conditions:

|                                  |                           |
|----------------------------------|---------------------------|
| Temperature of the 1st oven      | 210°C.                    |
| Speed of travel of the yarn      | 41 m/minute               |
| Speed of rotation of the spindle | 74,000 revolutions/minute |
| Temperature of the 2nd oven      | 215°C.                    |

Theoretical twist of the yarn 1,800 turns/meter

The yarn obtained in this example shows free portions which are shorter than in the preceding example, as is illustrated by FIG. 9.

#### EXAMPLE 7

The same procedure as in the two preceding examples is applied to the same yarn as in Example 1, under the following conditions:

|                                              |                           |
|----------------------------------------------|---------------------------|
| Temperature of the 1st oven                  | 215°C.                    |
| Speed of travel of the yarn through the oven | 41 m/minute               |
| Speed of rotation of the spindle             | 74,000 revolutions/minute |
| Temperature of the 2nd oven                  | 210°C.                    |

Theoretical twist of the yarn 1,800 turns/meter

The yarn obtained in this example has a very small number of very short free portions and its appearance is illustrated in FIG. 10.

#### EXAMPLE 8

To obtain a fancy effect yarn, the yarn obtained according to Example 4 is passed over an emery-covered surface which abrades the yarn and gives it the appearance shown schematically in FIG. 11.

#### EXAMPLE 9

In order to manufacture a "pile" yarn, the yarn obtained according to Example 5 is passed over a grinding wheel and a yarn of the appearance shown in FIG. 12 is obtained.

#### EXAMPLE 10

In order to form a yarn of "spun yarn" appearance, the yarn obtained in Example 6 is passed over a blade device which breaks the free portions formed on the surface of the yarn.

A fancy yarn having the appearance defined in FIG. 13 is thus obtained.

#### EXAMPLE 11

The yarn obtained in Example 7 is treated by means of an abrasive surface and the yarn illustrated in FIG. 5 14 is obtained.

#### EXAMPLE 12

A yarn identical to that of Example 1 is treated discontinuously by the process illustrated in FIG. 3, and 10 given a Z-twist of 1,250 turns/meter, and is then passed over a heating plate at a temperature of 240°C. at a speed of 7 meters/minute and wound up.

In a second phase, it is untwisted in the S-direction by 1,250 turns/meter and a yarn having the appearance 15 shown schematically in FIG. 15 is obtained.

#### EXAMPLE 13

Using the procedure of Example 1, the following sets of filaments are treated to form multi-filament yarns:

- 20 a. side by side polyethylene terephthalate and polypropylene terephthalate;  
 b. side by side polyacrylonitrile, and polyvinyl chloride; and  
 c. sheath, polyhexamethylene adipamide and core, 25 polyhexamethylene sebacamide.

Each of the above noted yarns has a compact effect substantially as shown in FIG. 4.

What we claim is:

1. A multi-filament yarn having an irregular surface and a twisted appearance, comprising at least two filaments, each filament having at least two components, each component having different softening temperatures, degradation temperatures or both, at least one of said components being thermoplastic, at least some of said filaments being bonded to each other at various points along the length of said yarn, the surface of said yarn having helical portions of random length, direction and pitch.  
 30 2. The yarn of claim 1, wherein said components are and a twisted appearance, comprising at least two filaments, each filament having at least two components, each component having different softening temperatures, degradation temperatures or both, at least one of said components being thermoplastic, at least some of said filaments being bonded to each other at various points along the length of said yarn, the surface of said yarn having helical portions of random length, direction and pitch.  
 35 3. The yarn of claim 1, wherein said filaments are co-axially formed of two different components in a sheath-core relationship, the sheath having a lower softening point than the core.  
 40 4. The yarn of claim 1, wherein a part of at least some of said filaments are bonded to each other at spaced intervals along said yarn.  
 45 5. The yarn of claim 1, wherein at least some of said filaments are bonded together only intermittently along the length of said yarn, and define free portions between these points which produce an effect.  
 50 6. The yarn of claim 5, wherein at least some of said filaments in said free portions are broken.

- 55 7. A process for obtaining an effect yarn comprising heating a multi-filament yarn having at least two filaments, each filament having at least two components having different softening temperatures, degradation temperatures or both, said filaments having at least one thermoplastic component, to a setting temperature at least sufficient to cause bonding of the component having the lowest softening temperature and insufficient to affect the textile characteristics of said component having the highest softening temperature, twisting said yarn and untwisting said yarn.  
 60 8. The process of claim 7, wherein said yarn is rapidly cooled after said heat treatment and prior to said untwisting treatment.

9. The process of claim 7, wherein said yarn is heated a second time after said yarn has untwisted.
10. The process of claim 7, wherein said yarn is additionally passed over a surface which causes some of the filaments of said yarn to break.
11. The process of claim 7, wherein the process is

continuous.

12. The process of claim 7, wherein the process is discontinuous.
13. The process of claim 7, wherein said twisting and untwisting is imparted by a false-twist spindle.

\* \* \* \* \*

10

15

20

25

30

35

40

45

50

55

60

65

UNITED STATES PATENT OFFICE  
CERTIFICATE OF CORRECTION

Patent No. 3,828,542 Dated August 13, 1974

Inventor(s) BOUTONNET, ET AL.

It is certified that error appears in the above-identified patent and that said Letters Patent are hereby corrected as shown below:

Please change the assignment information to read as follows:

-- Assignees: Rhone-Poulenc-Textile, S.A., Paris, France. --

Signed and Sealed this  
*twenty-third Day of September 1975*

[SEAL]

Attest:

**RUTH C. MASON**  
*Attesting Officer*

**C. MARSHALL DANN**  
*Commissioner of Patents and Trademarks*